

Aug. 28, 1923.

1,466,257

R. E. TALLEY

METHOD OF ANNEALING METALS

Filed June 9, 1919

Fig. 1.



Fig. 2.



WITNESSES:

H. J. Shelhamer  
W. Woodman.

INVENTOR

Randal E. Talley  
BY  
Meredith G. Barr  
ATTORNEY

## UNITED STATES PATENT OFFICE.

RANDAL E. TALLEY, OF IRWIN, PENNSYLVANIA, ASSIGNOR TO WESTINGHOUSE ELECTRIC & MANUFACTURING COMPANY, A CORPORATION OF PENNSYLVANIA.

## METHOD OF ANNEALING METAL.

Application filed June 9, 1919. Serial No. 302,837.

To all whom it may concern:

Be it known that I, RANDAL E. TALLEY, a citizen of the United States, and a resident of Irwin, in the county of Allegheny and 5 State of Pennsylvania, have invented a new and useful Improvement in Methods of Annealing Metals, of which the following is a specification.

My invention relates to a method of annealing metals, more particularly aluminum, and it has for its primary object the provision of a method which will insure better and more uniform results than any methods previously employed and known to me. 10 15 Heretofore, to the best of my knowledge, aluminum, in sheet or other forms, has been stacked in a large annealing furnace, often-times exceeding 30 feet in length, the annealing furnace has been sealed, and a fire 20 25 has been started to heat the furnace and keep it heated at the required temperature for a long period of time, ranging from 24 to 48 hours, in most instances.

The old method of annealing aluminum 30 35 has been very unsatisfactory because of non-uniformity of results. The large stacks of aluminum do not heat evenly, the outer portions being highly heated before the inner portions become appreciably heated, with 40 45 the result that the central portions of the sheets, or other forms being annealed, are hard.

Another fundamental objection to this method of annealing aluminum is that the 50 55 furnaces are usually heated by means of oil or gas flames and the products of combustion of such fuels combine with, or penetrate, the aluminum to such extent as to produce blisters on the surface of the metal being annealed. Porosity may also be caused thereby.

One of the objects of my present invention resides in providing a method of annealing aluminum by which the heating may 60 65 be constant and, consequently, the physical properties of the aluminum may be kept uniform and all blistering may be prevented.

A still further object of my invention resides in providing a method of heat treatment 70 75 which will not introduce impurities into the metal being annealed.

In order to insure a clear and accurate 80 85 understanding of my present method, reference may be had to the drawings illustrating one form of apparatus suitable for prac-

tising my invention. In the drawings, Fig. 1 is a sectional plan view of an electric furnace, and Fig. 2 is a vertical sectional view thereof.

While various types of electric furnaces 60 may be employed with equal facility, I have illustrated one particularly adapted to the purpose which comprises a furnace body 1, of fire brick, or other suitable material, open at its ends and provided with over-head, 65 longitudinally extending, heating elements 2. Any suitable form of conveyer, such as an inclined roller-table 3, may be provided for supplying the material to be annealed to the upper stretch of an endless conveyer 4, 70 of any suitable type, which extends throughout the length of the furnace. This conveyer 4 may preferably be of such character that its surfaces shall be smooth and uninterrupted to form proper support for the 75 aluminum sheets being annealed. A second inclined roller-table 5 may be disposed to receive the material as it passes from the furnace and to deposit it upon a cooling 80 conveyer 6, of any desired character.

In practising my invention, the aluminum to be annealed, which is preferably in the form of thin sheets, is supplied to the table 3 and fed by it to the conveyer 4 which is driven at a predetermined speed. The electric furnace is maintained at a constant temperature, suitable for the proper annealing 85 of the aluminum, which may be between 350° C. to 500° C. By this means, the aluminum is brought to the desired temperature 90 after which it passes from the furnace to the cooling conveyer 6 where it may cool naturally in the air or may be artificially cooled, as preferred.

My invention depends principally upon 95 the fact that aluminum may be successfully annealed by heating it to a certain definite temperature, such as 400° C., and that it need not be kept at this temperature for any considerable length of time. It is, therefore, 100 possible to anneal the aluminum during its brief passage through an electrically heated furnace, as above described.

The time required to properly anneal the aluminum will, of course, depend upon the 105 form of the material but tests made by me indicate that thin sheets of approximately 0.04 inch in thickness may be annealed in ten minutes or less. It will, therefore, be obvious that there is a great saving of 110

time by my process, with a consequent quick turn-over of material resulting in a saving of storage space. Furthermore, my method permits continuous annealing of the aluminum and, consequently, insures an uninterrupted supply of the annealed material.

As the heat of the electric furnace may be readily and accurately regulated and as only small quantities of the metal are in the furnace at any one time, great uniformity is insured, and the physical properties of the annealed metal are far superior to those of metal annealed by old methods.

There is no tendency of the metal to blister during its annealing in the electric furnace and, as the electric heat insures an inert atmosphere, there is no absorption of gases or other impurities.

Preferably the aluminum will be supplied to the furnace in single sheets although several sheets may be stacked upon each other if desired. For this reason, the heating elements of the furnace may be disposed only a fraction of an inch above the surface of the conveyor so that the volume of the heating chamber of the furnace is reduced to, in some instances, as low as one per cent of that of the furnaces now employed. This naturally results in a great saving of heat energy.

Although I have described my method

with particular reference to the annealing of aluminum, it will be appreciated that it may be employed for annealing other metals, if found suited for the purpose. It will also be understood that any suitable type of electric furnace and of conveyor structures may be employed. For these reasons, no limitations are to be imposed upon my invention other than those indicated in the claims.

I claim as my invention:

1. A method of annealing aluminum which comprises passing the aluminum through an electrically heated furnace at a predetermined speed.

2. A method of annealing aluminum which comprises continuously passing successive pieces of aluminum, at a predetermined rate, through an electric furnace heated to a predetermined degree.

3. A method of annealing aluminum which comprises successively supplying aluminum in small quantities to an electrically heated furnace, causing the aluminum so supplied to pass continuously through the furnace at a predetermined rate of speed, and cooling the aluminum as it passes from the furnace.

In testimony whereof, I have hereunto subscribed my name this 31st day of May, 1919.

RANDAL E. TALLEY.